

Aug. 5, 1924.

1,503,613

W. L. TAYLOR

PAPER MANUFACTURE

Filed Aug. 7, 1922



INVENTOR:

William L. Taylor

BY

Allen Allen

ATTORNEYS.

## UNITED STATES PATENT OFFICE.

WILLIAM L. TAYLOR, OF CINCINNATI, OHIO.

## PAPER MANUFACTURE.

Application filed August 7, 1922. Serial No. 580,057.

*To all whom it may concern:*

Be it known that I, WILLIAM L. TAYLOR, a citizen of the United States, and a resident of Cincinnati, in the county of Hamilton and State of Ohio, have invented certain new and useful Improvements in Paper Manufacture, of which the following is a full, clear, and exact description, reference being had to the accompanying drawings, forming part of this specification.

My invention relates to the manufacture of asphalt or bitumen pasted paper material, and to the processes involved in pasting the paper by means of the asphalt in such a way as to provide as perfect as possible a sheet for use in the production of bags and packages with the use of automatic machinery.

In a former application, Serial No. 551, 2018, filed by me on April 10, 1922, I describe a method of paper manufacture, in which gum streams are used along certain defined paths, patterns, or edges of asphalt pasted stock, so as to provide a non-asphaltic binder between the webs of paper along the lines through which the paper is to be cut in forming the bag, as well as the edges of the paper.

In that application I refer to cement as being used and in this application I desire to cover the use of materials other than what is generally known as cement, which materials have a lubricating quality on the cutting knives used in bag and package making machinery.

In some cases the use of cement or materials having a cementitious quality, but of non-asphaltic nature, will be necessary, and in some cases it will not be advisable to use this material.

I have found that for the best possible operation in high speed automatic machinery it is inadvisable to have a sheet which is more bulky at one point than another. This prevents a full grasp by the pressure rollers of clamp plates in the cutting machinery, and in doing so acts to permit the knives to tear the paper in cutting.

I have found that a water dissolved cement, which is about all that would be used in my first invention in this connection, as above identified, due to expense of other solvents, tends to bulk up the paper where it is cemented along the margins of the cemented band by the water getting into

the paper and flowing through it outside of the cemented band, so that it bulks up over the asphalt binder. Also I have found that the cemented band tends to have a reduced bulk over the asphalt portion of the paper and to give way under the pressure rolls, clamps, etc., of the cutting machines.

I have discovered also that usual cements do not have the lubricating quality that is desired under the cutting knives.

Thus in this invention I desire to cover the method of paper manufacture wherein there are lines, zones or patterns of material of bulk to maintain an even thickness sheet so far as possible, whether or not said materials have a cementing quality, so long as they are not of the quality of asphalt having tackiness sufficient to act as a binder between two plies of paper. In this one respect I desire to generically cover the invention set forth in my application above identified in this application rather than to pursue generic claims in the former one.

I accomplish the objects set forth and avoid the difficulties mentioned, by that certain process of paper manufacture to be hereinafter more specifically pointed out and claimed.

In the drawings,

Figure 1 represents a piece of pasted paper material formed with lines or bands of non-tacky asphalt or other substance.

Figure 2 is a cross section of Figure 1.

In the drawing I show two plies of paper 1 and 2, between which is a binding or cementing layer of tacky asphalt material 3 for purposes of moisture proofing.

Along the margins of the sheet are bands 4 of other material than the binding asphalt, and along desired lines running through the sheet are lines 5 of the same other material.

I prefer to use for the bands or streams, a material liquefiable by heat without solvent, and I apply the material in the manner set forth in my application above referred to. I also prefer to avoid materials which will tend to destroy the fiber mat of the paper, such as water-dissolved materials. I also prefer to use a material which has some solvent action on asphalt, so as to merge the continuous edges of tacky asphalt and the interposed or marginal bands, thereby preventing the asphalt from forming a bead along the margins thereof,

and getting an even thickness of the paper throughout, after it is formed into the double ply.

I also prefer that the material should have a lubricating quality on the cutting edges of knives in paper cutters used in forming bags and packages, thereby facilitating their work.

Such materials which I have successfully employed are paraffin, beeswax and a mixture of paraffin and asphalt. I have not gone beyond this range of materials in my preliminary work or commercial applications, but having above outlined the various points to be included within the function of the material used in the streams, bands, patterns or zones, it may well be that other products will serve the same purpose.

The resulting paper product is formed with two plies of paper, preferably, although the addition of further plies would not modify the fact that two plies, at least, are employed. The paper is cemented together by an asphalt which has resiliency and tackiness, so as to bind the plies fairly well together and form a layer of non-porous, moisture-resisting material throughout the body of the sheet.

The lines, etc., of other material may or may not act in a cementing capacity on the paper, but they do prevent the cutting knives of paper machinery having to pass through layers of asphalt body in slitting the paper for use in making desired articles therefrom.

The interlined material is of a quality by preference to result in forming a like bulk or caliper to the paper at the non-tacky lines, as has the main body of the paper. The edges of the sheet, as it is slit or formed at the paper mill, do not have the tacky asphalt extending therefrom.

The knives in cutting the paper pass through a substance which has a lubricating effect on them, and an even engagement of the paper by pressure rolls or clamps results in a proper cutting action of the knives. Foil or fabric could be used instead of paper, as in the former case.

Having thus described my invention, what I claim as new and desire to secure by Letters Patent, is:—

1. A web, comprising plies of paper, foil or fabric united into a web by a binding, interposed layer of tacky bituminous material, such as asphalt, with selected portions of the web, particularly the lines, where same is to be cut substantially free of the bituminous material, and having at such selected portions an interposed layer of other than tacky bitumen, said latter layer being of a solvent nature with the bitumen.

2. A web, comprising plies of paper, foil or fabric united into a web by a binding, interposed layer of tacky bituminous material, such as asphalt, with selected portions of the web, particularly the lines, where same is to be cut substantially free of the bituminous material, and having at such selected portions an interposed layer of other than tacky bitumen, said layer being of a waxy lubricating quality on cutting knives.

3. A process of forming narrow webs of asphalt pasted stock, which consists in first forming a wide web by uniting plies of paper, foil or fabric with an asphalt or related bitumen with said materials, substantially omitted along selected bands, lengthwise of the web, and with a material having a waxy lubricating quality on cutter knives interposed between the plies throughout said selected bands, and then cutting the wide web into narrow webs along the said bands.

WILLIAM L. TAYLOR.